



US006573643B1

(12) **United States Patent**  
**Kumar et al.**

(10) **Patent No.:** **US 6,573,643 B1**  
(b4) **Date of Patent:** **Jun. 3, 2003**

(54) **FIELD EMISSION LIGHT SOURCE**(75) Inventors: **Nalin Kumar**, Cherry Hill, NJ (US); **Chenggang Xie**, Phoenix, AZ (US)(73) Assignee: **SI Diamond Technology, Inc.**, Austin, TX (US)

(\*) Notice: Subject to any disclaimer, the term of this patent is extended or adjusted under 35 U.S.C. 154(b) by 98 days.

(21) Appl. No.: **09/677,361**(22) Filed: **Oct. 2, 2000****Related U.S. Application Data**

(63) Continuation-in-part of application No. 08/868,644, filed on Jun. 4, 1997, now Pat. No. 6,127,773, which is a continuation of application No. 08/071,157, filed on Jun. 2, 1993, now abandoned, which is a continuation-in-part of application No. 07/851,701, filed on Mar. 16, 1992, now Pat. No. 5,763,997, which is a continuation-in-part of application No. 08/456,453, filed on Jun. 1, 1995, now abandoned, which is a continuation-in-part of application No. 07/993,863, filed on Dec. 23, 1998, now abandoned.

(51) **Int. Cl. 7** ..... **H01J 1/30**(52) **U.S. Cl.** ..... **313/309; 313/496; 313/346 R**(58) **Field of Search** ..... 313/283, 309, 313/311, 336, 351, 496, 244, 346 R, 495(56) **References Cited****U.S. PATENT DOCUMENTS**

2,392,161 A \* 1/1946 Leverenz ..... 176/122

3,413,510 A \* 11/1968 Kerslake ..... 313/231  
4,345,181 A \* 8/1982 Shelton ..... 313/309  
5,345,141 A \* 9/1994 Moyer et al. ..... 313/495  
5,801,486 A \* 9/1998 Johnson et al. ..... 313/495  
6,008,575 A \* 12/1999 Kaftanov et al. ..... 313/484  
6,312,303 B1 \* 11/2001 Yaniv et al. ..... 445/24

**FOREIGN PATENT DOCUMENTS**

EP 845154 \* 11/1999  
JP 58218747 \* 12/1983 ..... H01J/61/54

\* cited by examiner

*Primary Examiner*—Ashok Patel(74) *Attorney, Agent, or Firm*—Kelly K. Kordzik; Winstead Sechrest & Minick P.C.(57) **ABSTRACT**

A field emission cathode for use in flat panel displays is described including a layer of conductive material and a layer of amorphic diamond film, functioning as a low effective work-function material, deposited over the conductive material to form emission sites. The emission sites each contain at least two sub-regions having differing electron affinities. Use of the cathode to form a computer screen is also described along with the use of the cathode to form a fluorescent light source.

**24 Claims, 2 Drawing Sheets**



FIG. 1



FIG. 2



FIG. 3



FIG. 4



FIG. 5



FIG. 6



FIG. 9



FIG. 7



FIG. 8

## FIELD EMISSION LIGHT SOURCE

This application is a continuation-in-part of U.S. patent application Ser. No. 08/868,644 now U.S. Pat. No. 6,127,773; filed on Jun. 4, 1997 which is a continuation of U.S. patent application Ser. No. 08/071,157 now abandoned filed on Jun. 2, 1993; which is a continuation-in-part of U.S. patent application Ser. No. 07/851,701 now abandoned filed on Mar. 16, 1992; which is a continuation-in-part of U.S. patent application Ser. No. 08/456,453 now U.S. Pat. No. 5,763,997 filed on Jun. 1, 1995; which is a continuation-in-part of U.S. patent application Ser. No. 07/993,863 now abandoned filed on Dec. 23, 1992.

## TECHNICAL FIELD OF THE INVENTION

This invention relates, in general, to flat field emission cathodes and, more particularly, to such cathodes which employ an amorphic diamond film having a plurality of emission sites situated on a flat emission surface.

## BACKGROUND OF THE INVENTION

Field emission is a phenomenon which occurs when an electronic field proximate the surface of an emission material narrows a width of a potential barrier existing at the surface of the emission material. This allows a quantum tunnelling effect to occur, whereby electrons cross through the potential barrier and are emitted from the material. This is as opposed to thermionic emission, whereby thermal energy within an emission material is sufficient to eject electrons from the material. Thermionic emission is a classical phenomenon, whereas field emission is a quantum mechanical phenomenon.

The field strength required to initiate field emission of electrons from the surface of a particular material depends upon that material's effective "work function." Many materials have a positive work function and thus require a relatively intense electric field to bring about field emission. Some materials do, in fact, have a low work function, or even a negative electron affinity, and thus do not require intense fields for emission to occur. Such materials may be deposited as a thin film onto a conductor, resulting in a cathode with a relatively low threshold voltage required to produce electron emissions.

In prior art devices, it was desirable to enhance field emission of electrons by providing for a cathode geometry which focussed electron emission at a single, relatively sharp point at a tip of a conical cathode (called a micro-tip cathode). These micro-tip cathodes, in conjunction with extraction grids proximate the cathodes, have been in use for years in field emission displays.

For example, U.S. Pat. No. 4,857,799, which issued on Aug. 15, 1989, to Spindt et al., is directed to a matrix-addressed flat panel display using field emission cathodes. The cathodes are incorporated into the display backing structure, and energize corresponding cathodoluminescent areas on a face plate. The face plate is spaced 40 microns from the cathode arrangement in the preferred embodiment, and a vacuum is provided in the space between the plate and cathodes. Spacers in the form of legs interspersed among the pixels maintain the spacing, and electrical connections for the bases of the cathodes are diffused sections through the backing structure. Spindt et al. employ a plurality of micro-tip field emission cathodes in a matrix arrangement, the tips of the cathodes aligned with apertures in an extraction grid over the cathodes. With the addition of an anode over the extraction grid, the display described in Spindt et al. is a triode (three terminal) display.

Unfortunately, micro-tips employ a structure which is difficult to manufacture, since the micro-tips have fine geometries. Unless the micro-tips have a consistent geometry throughout the display, variations in emission from tip to tip will occur, resulting in unevenness in illumination of the display. Furthermore, since manufacturing tolerances are relatively tight, such micro-tip displays are expensive to make.

For years, others have directed substantial effort toward solving the problem of creating cathodes which can be mass manufactured to tight tolerances, allowing them to perform with accuracy and precision. Another object of some of these prior art inventions was that they made use of emission materials having a relatively low effective work function so as to minimize extraction field strength.

One such effort is documented in U.S. Pat. No. 3,947,716, which issued on Mar. 30, 1976, to Fraser, Jr. et al., directed to a field emission tip on which a metal adsorbent has been selectively deposited. In a vacuum, a clean field emission tip is subjected to heating pulses in the presence of an electrostatic field to create thermal field build up of a selected plane. Emission patterns from this selected plane are observed, and the process of heating the tip within the electrostatic field is repeated until emission is observed from the desired plane. The adsorbent is then evaporated onto the tip. The tip constructed by this process is selectively faceted with the emitting planar surface having a reduced work function and the non-emitting planar surface as having an increased work function. A metal adsorbent deposited on the tip so prepared results in a field emitter tip having substantially improved emission characteristics. Unfortunately, as previously mentioned, such micro-tip cathodes are expensive to produce due to their fine geometries. Also, since emission occurs from a relatively sharp tip, emission is still somewhat inconsistent from one cathode to another. Such disadvantages become intolerable when many cathodes are employed in great numbers such as in a flat panel display for a computer.

As is evident in the above-described cathode structure, an important attribute of good cathode design is to minimize the work function of the material constituting the cathode. In fact, some substances such as alkali metals and elemental carbon in the form of diamond crystals display a low effective work function. Many inventions have been directed to finding suitable geometries for cathodes employing negative electron affinity substances as a coating for the cathode.

For instance, U.S. Pat. No. 3,970,887, which issued on Jul. 20, 1976, to Smith et al., is directed to a microminiature field emission electron source and method of manufacturing the same wherein a single crystal semiconductor substrate is processed in accordance with known integrated microelectronic circuit techniques to produce a plurality of integral, single crystal semiconductor raised field emitter tips at desired field emission cathode sites on the surface of a substrate in a manner such that the field emitters tips are integral with the single crystal semiconductor substrate. An insulating layer and overlying conductive layer may be formed in the order named over the semiconductor substrate and provided with openings at the field emission locations to form micro-anode structures for the field emitter tip. By initially appropriately doping the semiconductor substrate to provide opposite conductivity-type regions at each of the field emission locations and appropriately forming the conductive layer, electrical isolation between the several field emission locations can be obtained. Smith et al. call for a sharply-tipped cathode. Thus, the cathode disclosed in Smith et al. is subject to the same disadvantages as Fraser, Jr. et al.

U.S. Pat. No. 4,307,507, which issued on Dec. 29, 1981, to Gray et al., is directed to a method of manufacturing a field-emitter array cathode structure in which a substrate of single crystal material is selectively masked such that the unmasked areas define islands on the underlying substrate. The single crystal material under the unmasked areas is orientation-dependent etched to form an array of holes whose sides intersect at a crystal graphically sharp point.

U.S. Pat. No. 4,685,996, which issued on Aug. 11, 1987, to Busta et al., is also directed to a method of making a field emitter and includes an anisotropically etched single crystal silicon substrate to form at least one funnel-shaped protrusion on the substrate. The method of manufacturing disclosed in Busta et al. provides for a sharp-tipped cathode.

Sharp-tipped cathodes are further described in U.S. Pat. No. 4,885,636, which issued on Aug. 8, 1989, to Busta et al.

Yet another sharp-tipped emission cathode is disclosed in U.S. Pat. No. 4,964,946, which issued on Oct. 23, 1990, to Gray et al. Gray et al. disclose a process for fabricating soft-aligned field emitter arrays using a soft-leveling planarization technique, e.g. a spin-on process.

Even though they employ low effective work-function materials to advantage, sharp-tipped cathodes have fundamental problems when employed in a flat panel graphic display environment, as briefly mentioned above. First, they are relatively expensive to manufacture. Second, they are hard to manufacture with great consistency. That is, electron emission from sharp-tipped cathodes occurs at the tip. Therefore, the tip must be manufactured with extreme accuracy such that, in a matrix of adjacent cathodes, some cathodes do not emit electrons more efficiently than others, thereby creating an uneven visual display. In other words, the manufacturing of cathodes must be made more reliable so as to minimize the problem of inconsistencies in brightness in the display along its surface.

In Ser. No. 07/851,701, which was filed on Mar. 16, 1992, and entitled "Flat Panel Display Based on Diamond Thin Films," an alternative cathode structure was first disclosed. Ser. No. 07/851,701 discloses a cathode having a relatively flat emission surface as opposed to the aforementioned micro-tip configuration. The cathode, in its preferred embodiment, employs a field emission material having a relatively low effective work function. The material is deposited over a conductive layer and forms a plurality of emission sites, each of which can field-emit electrons in the presence of a relatively low intensity electric field.

Flat cathodes are much less expensive and difficult to produce in quantity because the fine, micro-tip geometry has been eliminated. The advantages of the flat cathode structure was discussed at length therein. The entirety of Ser. No. 07/851,701, which is commonly assigned with the present invention, is incorporated herein by reference.

A relatively recent development in the field of materials science has been the discovery of amorphic diamond. The structure and characteristics of amorphic diamond are discussed at length in "Thin-Film Diamond," published in the Texas Journal of Science, vol. 41, no. 4, 1989, by C. Collins et al. Collins et al. describe a method of producing amorphic diamond film by a laser deposition technique. As described therein, amorphic diamond comprises a plurality of micro-crystallites, each of which has a particular structure dependent upon the method of preparation of the film. The manner in which these micro-crystallites are formed and their particular properties are not entirely understood.

Diamond has a negative electron affinity. That is, only a relatively low electric field is required to distort the potential

barrier present at the surface of diamond. Thus, diamond is a very desirable material for use in conjunction with field emission cathodes. In fact, the prior art has employed crystalline diamond films to advantage as an emission surface on micro-tip cathodes.

In "Enhanced Cold-Cathode Emission Using Composite Resin-Carbon Coatings," published by S. Bajic and R. V. Latham from the Department of Electronic Engineering and Applied Physics, Aston University, Aston Triangle, Birmingham B4 7ET, United Kingdom, received May 29, 1987, a new type of composite resin-carbon field-emitting cathode is described which is found to switch on at applied fields as low as approximately  $1.5 \text{ MV m}^{-1}$ , and subsequently has a reversible I-V characteristic with stable emission currents of  $> 1 \text{ mA}$  at moderate applied fields of typically  $< 8 \text{ MV m}^{-1}$ . A direct electron emission imaging technique has shown that the total externally recorded current stems from a high density of individual emission sites randomly distributed over the cathode surface. The observed characteristics have been qualitatively explained by a new hot-electron emission mechanism involving a two-stage switch-on process associated with a metal-insulator-metal-insulator-vacuum (MIMIV) emitting regime. However, the mixing of the graphite powder into a resin compound results in larger grains, which results in fewer emission sites since the number of particles per unit area is small. It is preferred that a larger amount of sites be produced to produce a more uniform brightness from a low voltage source.

In "Cold Field Emission From CVD Diamond Films Observed In Emission Electron Microscopy," published by C. Wang, A. Garcia, D. C. Ingram, M. Lake and M. E. Kordesch from the Department of Physics and Astronomy and the Condensed Matter and Surface Science Program at Ohio University, Athens, Ohio on Jun. 10, 1991, there is described thick chemical vapor deposited "CVD" polycrystalline diamond films having been observed to emit electrons with an intensity sufficient to form an image in the accelerating field of an emission microscope without external excitation. The individual crystallites are of the order of 1–10 microns. The CVD process requires  $800^\circ \text{ C}$ . for the depositing of the diamond film. Such a temperature would melt a glass substrate.

The prior art has failed to: (1) take advantage of the unique properties of amorphic diamond; (2) provide for field emission cathodes having a more diffused area from which field emission can occur; and (3) provide for a high enough concentration of emission sites (i.e., smaller particles or crystallites) to produce a more uniform electron emission from each cathode site, yet require a low voltage source in order to produce the required field for the electron emissions.

## SUMMARY OF THE INVENTION

The prior art has failed to recognize that amorphic diamond, which has physical qualities which differ substantially from other forms of diamond, makes a particularly good emission material. Ser. No. 07/851,701 was the first to disclose use of amorphic diamond film as an emission material. In fact, in the preferred embodiment of the invention described therein, amorphic diamond film was used in conjunction with a flat cathode structure to result in a radically different field emission cathode design.

The present invention takes the utilization of amorphic diamond a step further by depositing the amorphic diamond in such a manner so that a plurality of diamond micro-crystallite regions are deposited upon the cathode surface

such that at each region (pixel) there are a certain percentage of the crystals emerging in an  $SP^2$  configuration and another percentage of the crystals emerging in an  $SP^3$  configuration. The numerous  $SP^2$  and  $SP^3$  configurations at each region result in numerous discontinuities or interface boundaries between the configurations, with the  $SP^2$  and  $SP^3$  crystallites having different electron affinities.

Accordingly, to take advantage of the above-noted opportunities, it is a primary object of the present invention to provide an independently addressable cathode, comprising a layer of conductive material and a layer of amorphic diamond film, functioning as a low effective work-function material, deposited over the conductive material, the amorphic diamond film comprising a plurality of distributed localized electron emission sites, each sub-site having an plurality of sub-regions with differing electron affinities between sub-regions.

In a preferred embodiment of the present invention, the amorphic diamond film is deposited as a relatively flat emission surface. Flat cathodes are easier and, therefore, less expensive to manufacture and, during operation of the display, are easier to control emission therefrom.

A technical advantage of the present invention is to provide a cathode wherein emission sites have electrical properties which include discontinuous boundaries with differing electron affinities.

Another technical advantage of the present invention is to provide a cathode wherein emission sites contain dopant atoms.

Yet another technical advantage of the present invention is to provide a cathode wherein a dopant atom is carbon.

Yet a further technical advantage of the present invention is to provide a cathode wherein emission sites each have a plurality of bonding structures.

Still yet another technical advantage of the present invention is to provide a cathode wherein one bonding structure at an emission site is  $SP^3$ .

Still a further technical advantage of the present invention is to provide a cathode wherein each emission site has a plurality of bonding orders, one of which is  $SP^3$ .

Another technical advantage of the present invention is to provide a cathode wherein emission sites contain dopants of an element different from a low effective work-function material. In the case of use of amorphic diamond as the low effective work-function material, the dopant element is other than carbon.

Still another technical advantage of the present invention is to provide a cathode wherein emission sites contain discontinuities in crystalline structure. The discontinuities are either point defects, line defects or dislocations.

The present invention further includes novel methods of operation for a flat panel display and use of amorphic diamond as a coating on an emissive wire screen and as an element with a cold cathode fluorescent lamp.

In the attainment of the above-noted features and advantages, the preferred embodiment of the present invention is an amorphic diamond film cold-cathode comprising a substrate, a layer of conductive material, an electronically resistive pillar deposited over the substrate and a layer of amorphic diamond film deposited over the conductive material, the amorphic diamond film having a relatively flat emission surface comprising a plurality of distributed micro-crystallite electron emission sites having differing electron affinities.

The foregoing has outlined rather broadly the features and technical advantages of the present invention in order that

the detailed description of the invention that follows may be better understood. Additional features and advantages of the invention will be described hereinafter which form the subject of the claims of the invention. It should be appreciated by those skilled in the art that the conception and the specific embodiment disclosed may be readily utilized as a basis for modifying or designing other structures for carrying out the same purposes of the present invention. It should also be realized by those skilled in the art that such equivalent constructions do not depart from the spirit and scope of the invention as set forth in the appended claims.

#### BRIEF DESCRIPTION OF THE DRAWINGS

For a more complete understanding of the present invention, and the advantages thereof, reference is now made to the following descriptions taken in conjunction with the accompanying drawings, in which:

FIG. 1 is a cross-sectional representation of the cathode and substrate of the present invention;

FIG. 2 is a top view of the cathode of the present invention including emission sites;

FIG. 3 is a more detailed representation of the emission sites of FIG. 2;

FIG. 4 is a cross-sectional view of a flat panel display employing the cathode of the present invention;

FIG. 5 is a representation of a coated wire matrix emitter;

FIG. 6 is a cross-sectional view of a coated wire;

FIG. 7 is a side view of a fluorescent tube employing the coated wire of FIG. 6;

FIG. 8 is a partial section end view of the fluorescent tube of FIG. 7; and

FIG. 9 is a computer with a flat-panel display that incorporates the present invention.

#### DETAILED DESCRIPTION OF THE INVENTION

Turning now to FIG. 1, shown is a cross-sectional representation of the cathode and substrate of the present invention. The cathode, generally designated 10, comprises a resistive layer 11, a low effective work-function emitter layer 12 and an intermediate metal layer 13. The cathode 10 sits on a cathode conductive layer 14 which, itself, sits on a substrate 15. The structure and function of the layers 11, 12, 13 of the cathode 10 and the relationship of the cathode 10 to conductive layer 14 and substrate 15 are described in detail in related application Ser. No. 07/851,701, which is incorporated herein by reference.

Turning now to FIG. 2, shown is a top view of the cathode 10 of FIG. 1. The emitter layer 12 is, in the preferred embodiment of the present invention, amorphic diamond film comprising a plurality of diamond micro-crystallites in an overall amorphous structure. The micro-crystallites result when the amorphic diamond material is deposited on the metal layer 13 by means of laser plasma deposition, chemical vapor deposition, ion-beam deposition, sputtering, low temperature deposition (less than 500 degrees Centigrade), evaporation, cathodic arc evaporation, magnetically separated cathodic arc evaporation, laser acoustic wave deposition or similar techniques or a combination of the above whereby the amorphic diamond film is deposited as a plurality of micro-crystallites. One such process is discussed within "Laser Plasma Source of Amorphic Diamond," published by the American Institute of Physics, January 1989, by C. B. Collins, et al.

The micro-crystallites form with certain atomic structures which depend on environmental conditions during deposition and somewhat on chance. At a given environmental pressure and temperature, a certain percentage of crystals will emerge in an  $SP^2$  (two-dimensional bonding of carbon atoms) configuration. A somewhat smaller percentage, however, will emerge in an  $SP^3$  (three-dimensional bonding) configuration. The electron affinity for diamond micro-crystallites in an  $SP^3$  configuration is less than that for carbon or graphite micro-crystallites in an  $SP^2$  configuration. Therefore, micro-crystallites in the  $SP^3$  configuration have a lower electron affinity, making them "emission sites." These emission sites (or micro-crystallites with an  $SP^3$  configuration) are represented in FIG. 2 as a plurality of black spots in the emitter layer 12.

The flat surface is essentially a microscopically flat surface. A particular type of surface morphology, however, is not required. But, small features typical of any polycrystalline thin film may improve emission characteristics because of an increase in enhancement factor. Certain micro-tip geometries may result in a larger enhancement factor and, in fact, the present invention could be used in a micro-tip or "peaked" structure.

Turning now to FIG. 3, shown is a more detailed view of the micro-crystallites of FIG. 2. Shown is a plurality of micro-crystallites 31, 32, 33, 34, for example. Micro-crystallites 31, 32, 33 are shown as having an  $SP^2$  configuration. Micro-crystallite 34 is shown as having an  $SP^3$  configuration. As can be seen in FIG. 3, micro-crystallite 34 is surrounded by micro-crystallites having an  $SP^2$  configuration.

There are a very large number of randomly distributed localized emission sites per unit area of the surface. These emission sites are characterized by different electronic properties of that location from the rest of the film. This may be due to one or a combination of the following conditions:

- 1) presence of a doping atom (such as carbon) in the amorphous diamond lattice;
- 2) a change in the bonding structure from  $SP^2$  to  $SP^3$  in the same micro-crystallite;
- 3) a change in the order of the bonding structure in the same micro-crystallite;
- 4) an impurity (perhaps a dopant atom) of an element different from that of the film material;
- 5) an interface between the various micro-crystallites;
- 6) impurities or bonding structure differences occurring at the micro-crystallite boundary; or
- 7) other defects, such as point or line defects or dislocations.

The manner of creating each of the above conditions during production of the film is well known in the art.

One of the above conditions for creating differences in micro-crystallites is doping. Doping of amorphic diamond thin film can be accomplished by interjecting elemental carbon into the diamond as it is being deposited. When doping with carbon, micro-crystallites of different structures will be created statistically. Some micro-crystallites will be n-type. Alternatively, a non-carbon dopant atom could be used, depending upon the desired percentage and characteristics of emission sites. Fortunately, in the flat panel display environment, cathodes with as few as 1 emission site will function adequately. However, for optimal functioning, 1 to 10 n-type micro-crystallites per square micron are desired. And, in fact, the present invention results in micro-crystallites less than 1 micron in diameter, commonly 0.1 micron.

Emission from the cathode 10 of FIG. 1 occurs when a potential difference is impressed between the cathode 10 and an anode (not shown in FIG. 1) which is separated by some small distance from the cathode 10. Upon impression of this potential, electrons are caused to migrate to the emission layer 12 of the cathode 10.

In the example that follows, the condition that will be assumed to exist to create micro-crystallites of different work function will be a change in the bonding structure from  $SP^2$  to  $SP^3$  in the same micro-crystallites (condition 3 above). With respect to the emission sites shown in FIGS. 2 and 3, micro-crystallites having an  $SP^3$  configuration have a lower work-function and electron affinity than micro-crystallites having an  $SP^2$  configuration. Therefore, as voltage is increased between the cathode 10 and anode (not shown), the voltage will reach a point at which the  $SP^3$  micro-crystallites will begin to emit electrons. If the percentage of  $SP^3$  micro-crystallites on the surface of the cathode 10 is sufficiently high, then emission from the  $SP^3$  micro-crystallites will be sufficient to excite the anode (not shown), without having to raise voltage levels to a magnitude sufficient for emission to occur from the  $SP^2$  micro-crystallites. Accordingly, by controlling pressure, temperature and method of deposition of the amorphic diamond film in a manner which is well-known in the art,  $SP^3$  micro-crystallites can be made a large enough percentage of the total number of micro-crystallites to produce sufficient electron emission.

Turning now to FIG. 4, shown is a cross-sectional view of a flat panel display employing the cathode of the present invention. The cathode 10, still residing on its cathode conductive layer 14 and substrate 15 as in FIG. 1, has been mated to an anode, generally designated 41 and comprising a substrate 42, which in the preferred embodiment is glass. The substrate 42 has an anode conductive layer 43 which, in the preferred embodiment, is an indium tin oxide layer. Finally, a phosphor layer 44 is deposited on the anode conductive layer to provide a visual indication of electron flow from the cathode 10. In other words, when a potential difference is impressed between the anode 41 and the cathode 10, electrons flowing from the cathode 10 will flow toward the anode conductive layer 43 but, upon striking the phosphor layer 44, will cause the phosphor layer to emit light through the glass substrate 42, thereby providing a visual display of a type desirable for use in conjunction with computers or other video equipment. The anode 41 is separated by insulated separators 45, 46 which provide the necessary separation between the cathode 10 and the anode 41. This is all in accordance with the device described in Ser. No. 07/851,701.

Further, in FIG. 4, represented is a voltage source 47 comprising a positive pole 48 and a negative pole 49. The positive pole is coupled from the source 47 to the anode conductive layer 43, while the negative pole 49 is coupled from the source 47 to the cathode conductive layer 14. The device 47 impresses a potential difference between the cathode 10 and the anode 41, causing electron flow to occur between the cathode 10 and the anode 41 if the voltage impressed by the source 47 is sufficiently high.

Turning now to FIG. 9, there is illustrated computer 90 with associated keyboard 93, disk drive 94, hardware 92 and display 91. The present invention may be employed within display 91 as a means for providing images and text. All that is visible of the present invention is anode 41.

Turning now to FIG. 5, shown is a representation of a coated wire matrix emitter in the form of a wire mesh, generally designated 51. The wire mesh 51 comprises a

plurality of rows and columns of wire which are electrically joined at their intersection points. The wire mesh 51 is then coated with a material having a low effective work-function and electron affinity, such as amorphic diamond, to thereby produce a wire mesh cathode for use in devices which previously used an uncoated wire or plate cathode and application of a high current and potential difference to produce incandescence and a flow of electrons from the mesh to an anode. By virtue of the amorphic diamond coating and its associated lower work function, incandescence is no longer necessary. Therefore, the wire mesh 51 cathode can be used at room temperature to emit electrons.

Turning now to FIG. 6, shown is a cross-section of a wire which has been coated with a material having a low work-function and electron affinity. The wire, designated 61, has a coating 62 which has been deposited by laser plasma deposition, or any one of the other well-known techniques listed above to thereby permit the coating 62 to act as a cold cathode in the same manner as the cathodes described in FIGS. 1-5.

Coating 62 may also be a carbon film deposited using chemical vapor deposition, and other techniques of an equivalent nature, such as disclosed in U.S. patent application Ser. No. 08/859,960 and U.S. patent application Ser. No. 08/910,604, which are hereby incorporated by reference herein. Such a carbon film may comprise several different types of structures, including carbon flakes as disclosed in U.S. patent application Ser. No. 07/642,955 or carbon nanotubes such as disclosed in U.S. patent application Ser. No. 09/356,145 and 60/185,222, which are hereby incorporated by reference herein.

Turning now to FIG. 7, shown is one application of the wire 61 in which the coated wire 61 functions as a conductive filament and is surrounded by a glass tube 72, functioning as an anode and which has an electrical contact 73 to thereby produce a fluorescent tube. The tube functions in a manner which is analogous to the flat panel display application discussed in connection with FIGS. 1-5, that is, a potential difference is impressed between the wire 61 (negative) and the tube 72 sufficient to overcome the space-charge between the cathode wire 61 and the tube anode 72. Once the space-charge has been overcome, electrons will flow from emission site SP<sup>3</sup> micro-crystallites in the coating 62.

Turning now to FIG. 8, shown is a partial section end view of the fluorescent tube 71 of FIG. 7. Shown again are the wire 61 and the coating 62 of FIG. 6 which, together, form a low effective work-function cathode in the fluorescent tube 71. The glass tube 72 of FIG. 7 comprises a glass wall 81 on which is coated an anode conductive layer 82. The anode conductive layer 82 is electrically coupled to the electrical contact 73 of FIG. 7. Finally, a phosphor layer 83 is deposited on the anode conductive layer 82. When a potential difference is impressed between the cathode wire 61 and the anode conductive layer 82, electrons are caused to flow between the emitter coating 82 and the anode conductive layer 82. However, as in FIG. 4, the electrons strike the phosphor layer 83 first, causing the phosphor layer 83 to emit photons through the glass wall 81 and outside the fluorescent tube 71, thereby providing light in a manner similar to conventional fluorescent tubes. However, because the fluorescent tube of FIGS. 7 and 8 employs a cathode having a low effective work-function emitter, such as amorphic diamond film, the fluorescent tube does not get warm during operation. Thus, the energy normally wasted in traditional fluorescent tubes in the form of heat is saved. In addition, since the heat is not produced, it need not be later removed by air conditioning.

Although the present invention and its advantages have been described in detail, it should be understood that various changes, substitutions and alterations can be made herein without departing from the spirit and scope of the invention as defined by the appended claims.

What is claimed is:

1. A fluorescent light source, comprising:  
a layer of amorphic diamond film deposited over a conductive filament, said amorphic diamond film comprising a plurality of electron emission sites, each electron emission site having a plurality of sub-regions; and  
an anode surrounding said filament and said amorphic diamond film, said anode radiating light in response to receipt of electrons emitted by said electron emission sites.
2. The light source as recited in claim 1 wherein said emission surface is relatively flat.
3. The light source as recited in claim 1 wherein said emission sites at said emission surface are relatively flat.
4. The light source as recited in claim 1 wherein said sites have at least two different electron affinities.
5. The light source as recited in claim 1 wherein each said site is under 1 micron in diameter.
6. The light source as recited in claim 1 wherein said emission sites contain dopant atoms.
7. The light source as recited in claim 6 wherein said dopant atoms are carbon.
8. The light source as recited in claim 1 wherein said sub-regions each have at least two different bonding structures.
9. The light source as recited in claim 6 wherein one of said bonding structures is SP<sup>3</sup>.
10. The light source as recited in claim 1 wherein said anode comprises an outer transparent layer.
11. The light source as recited in claim 10 wherein said outer transparent layer is composed of glass.
12. The light source as recited in claim 10 wherein said outer transparent layer is hermetically sealed about said filament to thereby define a chamber and gap between said outer transparent layer and said filament.
13. The light source as recited in claim 1 wherein said anode comprises an inner light-emitting layer.
14. The light source as recited in claim 13 wherein said inner light-emitting layer is composed of phosphorescent material.
15. The light source as recited in claim 1 wherein said anode comprises a conductive layer located between an outer, transparent layer and an inner light-emitting layer.
16. The light source as recited in claim 15 wherein said conductive layer is composed of indium-tin oxide.
17. A light source comprising:  
a field emitter deposited over a conductive filament; and  
an anode surrounding said filament, said anode operable for emitting light in response to receipt of electrons from said field emitter deposited over said conductive filament.
18. The light source as recited in claim 17, wherein the anode comprises an outer transparent layer.
19. The light source as recited in claim 18, wherein said outer transparent layer is hermetically sealed about said filament to thereby define a chamber and gap between said outer transparent layer and said filament.
20. The light source as recited in claim 19, wherein said anode comprises a light-emitting layer.
21. The light source as recited in claim 20, wherein said light-emitting layer is composed of a phosphorescent material.

**22.** The light source as recited in claim **17**, wherein the field emitter comprises a carbon film.

**23.** The light source as recited in claim **17**, wherein said field emitter comprises carbon flakes.

**24.** The light source as recited in claim **17**, wherein the field emitter comprises carbon nanotubes.

\* \* \* \* \*